# EUROPEAN PATENT SPECIFICATION

(11) **EP 1 546 449 B1**
(45) Date of publication and mention of the grant of the patent: **31.10.2018**
(21) Application number: 03791172.4
(22) Date of filing: 01.09.2003
(51) Int. Cl.: D07B 1/16, D07B 7/16

(54) **A HIGH-STRENGTH LIGHT-WEIGHT ROPE WITH A SHAPED CORE**
HOCHFESTES LEICHTES SEIL MIT PROFILIERTER SEELE
CORDAGE LEGER HAUTEMENT RESISTANT POURVU D'UNE AME FACONNEE

(30) Priority: 30.08.2002 IS 653602
(43) Date of publication of application: 29.06.2005
(73) Proprietor: Hampidjan HF., 110 Reykjavik (IS)
(72) Inventor: ERLENDSSON, Hjortur, IS-201 Kopavogur (IS)
(74) Representative: Fridriksson, Einar Karl
(86) International application number: PCT/IS2003/000025
(87) International publication number: WO 2004/020732

(56) References cited:
- EP-A- 1 022 377
- EP-A- 1 033 435
- WO-A-00/50687
- DE-B- 1 073 677
- GB-A- 2 028 885
- GB-A- 2 266 322
- US-A- 2 284 728
- US-A- 3 686 855
- US-A- 4 378 725

## Description

### Field of the invention

The present invention relates to a rope with high cross-sectional symmetry having high stiffness and breaking strength.

### Background

Various types of ropes and cables exist for different operations. In some operations ropes are desired, that are twisted and braided with high breaking strength and simultaneously with low mass density. With improving technology in producing fibres (such as Aramids, Liquid Crystal Polymers, PBO and Ultra High Molecular Weight Polyethylene), ropes with high breaking strength have been produced, with a breaking strength that is greater than for steel wire of the same diameter. Furthermore, the weight of such ropes is only one-sixth of the weight of a same size steel wire. One of the advantages of such ropes is that they are much easier to handle than steel wire. Applications for such ropes are e.g. in fishing with nets and trawls, where the ropes are used for back strop attachments, bridles and sweep lines.

The problem with such ropes is that openings are formed in between the strands. Those openings or vacancies allow the strands to move and the cross-sectional stability is therefore low if the vacancies are not filled out.

A common type of ropes used for trawl warps, bridles and sweep lines are twisted steel wire ropes. In twisted steel wire rope the most common construction is based on seven strands where one is in the centre and the remaining six are twisted around the centre strand. The centre strand is therefore acting as a core filling up the void. In steel wire ropes the core is often made from other materials like a bundle of fibres, twine or even synthetic ropes. As the steel wire is very stiff and harder than such softer materials, the core will be clenched and fill eventual voids. The result is that these soft core steel ropes have high strength, excellent abrasion resistance, circular cross-section and the stiffness is high in axial as well as in radial directions. One of the advantages of using steel wire rope for warps is how accurately it can be wound on drum winches. This prevents tangling on the drum as the rope will not be buried down between previous layers, and ropes in the same layer will not cross each other and damage the underlying rope. Despite this, there are some drawbacks using steel wire ropes. The steel wires are very heavy and difficult to work with and the lifetime is often limited due to corrosion and bending fatigue. The weight of the rope once in the sea can make it difficult to tow trawls and particularly when the trawl is used in mid water or even close to the surface due to the high sinking force created by the high density of the warp.

This problem has partly been solved by providing synthetic fibre ropes with a stiff core that adds considerable stiffness to the rope without adding much to the diameter. Their strength is close to or higher than that of steel wire ropes of the same diameter. These stiff-core fibre ropes have been available for many years. In such fibre ropes the fibre is soft and the core is similar material as the covering strands, but they will not be clenched in the same way as in steel wire ropes. If the core is stiff, the inside of the fibre will adjust to the contours of the core but not vice-versa. Therefore it is difficult to completely fill out the voids in fibre ropes and at the same time preserve the inside contour unless the core material is much softer than the fibre strands surrounding the core. Core material that is softer than the surrounding fibre material will therefore not enhance the stiffness of the rope.

US-A-4378725 discloses a method for producing a sealed rope of braided or twisted filaments. Heat-shrinkable filaments are braided or twisted about a core of a thermoplastic material to form a rope and the rope is placed under tension and treated to cause the thermoplastic core material to melt. Simultaneously the rope is maintained at a temperature sufficient to cause the heat-shrinkable filaments to shrink but not to melt, whereby the shrinking of the filaments, while the rope is under tension, reduces the cross section of the rope and causes the material to penetrate into the openings between and to surround and seal the filaments of the rope.

DE-B-10 73 677 relates to a curtain cord and a construction thereof.

EP-A-1033435 relates to a composite cord for reinforcement of elastomers comprising a core of a high polymer material, a first layer of steel filaments twisted around said core and a second layer of steel filaments twisted around said first layer. The polymer material is present in a sufficient volume to create gaps between adjacent filaments of the first layer and possibly also between the filaments of the second layer. The composite cord is characterised by a decreased fretting of the steel filaments.

US-A-3 686 855 relates to a cable with a solid core made of a relatively incompressible thermoplastic material.

WO-A-00/50687 relates to a low stretch elevator rope in which a plastic core has a central strength member that does not increase the weight of the rope by more than 5 %. Moreover, the plastic core has a diameter exceeding 50 % of the diameter of the rope, when measured prior to winding steel strands onto the core. The steel strands that are wound around the core are conventional and are so wound that the plastic material of the core essentially fills the inner interstices between the steel strands.

There is a need for a construction of a fibre rope, which gives it increased form stability.

### Description of the invention

The object of the present invention is to provide a strong rope by implementing a stiff core in a rope jacket in such a way that the core will preserve its stiffness and fill out the inside vacancies within the rope permanently. Braiding a fibre rope around a core which is made of thermoplastic material, can accomplish this. During the production process the rope is heated up and stretched in such a way that it will be permanently elongated. The thermoplastic core goes through a transition from a first solid phase to a second phase (typically a liquid or semi-liquid phase) and back to the solid phase by means of heating. During the second phase the core material will adapt to the void space within the rope jacket in which it is enclosed. The rope is then cooled down under tension until the core has regained its solid phase. To control the movement of the thermoplastic material in the liquid phase, it is covered by a sheet layer, e.g. overbraid, which has a higher softening point than the core material.

It will be particularly appreciated that ropes of the present invention have sufficient strength for use as towing wires for towing fish trawls, where conventionally much heavier steel wires have been used, which are sensitive to corrosion.

According to a first aspect, the present invention relates to a rope having high stiffness and breaking strength, comprising a core, and at least one jacket enclosing the core, wherein the high breaking strength is obtained by changing the phase condition of the core and optionally said at least one jacket from a first phase condition to a second phase condition while stretching the rope, thereby obtaining a relative movement of said at least one jacket layer and the core, so that the vacancies between the core and jacket are eliminated. A rope with stiffness and high breaking strength is thus obtained.

The core comprises a core material and a sheet layer, e.g. braided cover, enclosing said core material. Thereby it is prevented that the core material diffuses, in the second phase condition, towards the surface of the at least one sheet layer/jacket. The core material may be selected from any of a number of suitable thermoplastic materials (i.e., materials that become reversibly softer when heated and retain original properties (hardness) when cooled down). Preferably, the core is made of a plastic material, such as typically a thermoplastic polymer, a suitable polymer can be selected e.g. from nylon, olefin, or high-density polyethylene (HDPE), chlorinated polyethylene (CPE), polyester, or a combination thereof.

In certain useful embodiments, the core comprises additionally a central inner core (or "strength member") with different material properties than the main core material, for added strength and/or stiffness. The central inner core is preferably made from a fibre thread or filament, twinned or braided, from a suitable polymer, a single thread or metal wire, e.g. a lead or steel wire.

As mentioned, the first phase condition is a solid phase condition for both the core and the jacket. In preferred embodiments, the rope is treated such that the phase of the core changes while the phase conditions of the jacket remain unchanged. The second phase condition for the core is preferably a liquid phase condition but may also be an intermediate phase (semi-liquid phase) or a mixture of a liquid and solid phase, e.g. such that substantially all of the core is in a liquid or semi-liquid phase, though some parts/filaments may remain solid or semi-solid. In certain embodiments, the phase condition of the jacket is altered but generally however, the jacket remains substantially solid during the processing. (In these embodiments, a portion of the jacket, e.g. filaments or threads with a lower softening point than the main strands of the jacket, go through a phase transition and diffuse further in between the main strands of the jacket.)

The at least one jacket layer is preferably made of a plurality of strands where each strand typically is a bundle of fibre filaments, threads or yarns; the jacket is braided in such a way that the strands form at least a three-strand laid rope, such as a four- or six-strand laid rope. However, other arrangements are as well workable for the rope of the invention, hence, the strands may form a strand braided rope, with, e.g. 6, 8, 10, 12, 14, 16, 18, 20, 24, 28 or 32 strands braided.

In other embodiments more than a jacket is used, i.e. a sheet layer with a plurality of strands (e.g. 3, 4, or 6) and one or more outer jackets of strands, each outer jacket comprising a plurality of strands, such as described above.

The jacket may be made of one or more suitable materials, typically from one or more polymer fibre material such as but not limited to nylon, polyethylene, including high-density and ultra high-molecular weight polyethylene (e.g. Dyneema™ (DSM, Herleen, Netherlands)), aramids, liquid crystal polymers, PBO (polybenzoxazole polymer) or polyester, and any combination thereof, such combinations may also comprise steel wires or in a certain embodiment the jacket additionally comprises thermoplastic fibre threads, that during heating will soften or melt to blend in with the bulk material of the jacket.

The jacket is in certain embodiments enclosed by a cover which may be braided, coextruded or pulltruded and is preferably from a material selected from any of the materials listed above or a combination thereof (such as, e.g., from nylon, olefin, polypropylene, thermoplastic filaments, polyester, aramids, liquid crystal Polymers, PBO and polyethylene, including Ultra High Molecular Weight Polyethylene, (e.g. Dyneema™), and any combination thereof).

Furthermore, in order to enhance the strength of the at least one jacket, the threads and the strands in the at least one jacket are preferably internally fixed together. The force is thereby divided between all the strands and their threads, which co-operate. In order to increase the strength of the rope further, the at least one sheet layer is elongated such that the fibres in said at least one sheet layer have equal length. The strength is therefore not imposed on one or several fibres but on all the fibres. Such internal fixing may be obtained by contacting (impregnating) the jacket (optionally with the core mounted inside) with an adhesion material, such as preferably polyurethane or another material with similar suitable properties, e.g. by immersion, or by other suitable techniques such as spraying or using wet rollers.

The changing of the phase condition is by heating the core and optionally said at least one jacket. Preferably, the temperature for the phase change is in the range of 50-180°C, and preferably in the range of 100-130°C, or in the range of 110-120°C, such as, e.g., about 110, 112, or 115°C. The exact temperature or temperature range will, however, depend on the material or combination of materials comprised in the core, and their properties and softening point(s).

In other embodiments of the present invention, further means for coverbraiding the rope are used, mainly in order to increase the lifetime of the rope.

The relative movement of said at least one jacket and the core is effected through elongating lengthwise said at least one jacket layer, and optionally also the core. The elongation results in that the at least one jacket layer is clenched widthwise (cross-sectional), such that the core material when softened fills up in vacancies between the core and said at least one jacket layer. The cross- sectional symmetry of the rope may after the clenching be circular. However, other cross section symmetries are also possible.

According to a second aspect, the present invention provides a method for producing a rope with high stiffness and breaking strength, such as described above, the method comprising the steps of:
- providing a thermoplastic core in a solid phase condition,
- enclosing the core within a sheet layer that has a higher softening point than the core material,
- braiding about the core and the sheet layer at least one jacket,
- changing the phase condition of the core from the first solid phase condition to a second phase condition by heating, and
- simultaneously stretching said at least one jacket and the core in such a way that the rope becomes permanently elongated,
- subsequently cooling down the rope under tension until the core has regained its solid phase,
wherein the simultaneously stretching of the rope under an appropriate temperature is adapted to elongate the rope permanently and to eliminate vacancies between the core, the sheet layer, and the jacket so that a high stiffness and breaking strength is obtained and axial and radial stiffness are achieved.

All general features relating to the method and components of the rope (the core, the jacket, the phase conditions, stretching and the relative movement) is as described above.

In one preferred embodiment of the method the at least one jacket layer and optionally the core are brought in contact with an adhesion material as described above, so that the fibres in the sheet layer are internally joined together prior to the changing of the phase condition of the core. Polyurethane, which optionally can be diluted in aqueous solution, is preferred as an adhesion material.

Preferably the method further comprises removing the excess of said adhesion material and/or optionally moisture from said at least one jacket layer and the core prior to the stretching step.

### Detailed description

In the following the present invention, and in particular preferred embodiments thereof, will be described in greater detail in connection with the accompanying drawings in which,
Fig. 1 shows the core as a cylindrical bar but other cross-sectional shapes may equally be used as the core is reshaped during the production process according to the invention.
Fig. 2 shows the core as well but in the centre there is a strength member which can be useful for some thermoplastic core materials, as discussed herein.
Fig. 3 is a view of the core with a surrounding sheet from a material, which has higher thermal stability than the core material. This sheet can be co-extruded, pulltruded, wrapped, twisted or overbraided or made by a combination of two or more of said methods.
Fig.4 is showing the rope jacket around the core. The particular jacket illustrated in the drawing is a braided rope jacket. Each strand 5 is a twisted bundle of filaments or yarns.
Fig. 5 shows the core unravelled after the phase change process. The pattern is created by the clenching and elongation during the phase shifts of the core material.
Fig. 6 shows a view of a processed rope with a sheet cover. The cover can be co-extruded, pulltruded, wrapped, twisted or overbraided or made by a combination of two or more of said methods.

The core 1 is extruded with or without a strength member 2 in the middle. The material used is thermoplastic material of any kind but preferably a polymer. The core is cooled down until it reaches solid state. A sheet layer 3 is applied with a co-extrusion, pulltrusion, wrapping, twisting or overbraiding or a multiple or combination of the methods. The function of the sheet layer 3 is to prevent uncontrolled flow of the liquid or semi-liquid core during processing. In some cases not according to the invention, it is desirable to have the core flowing out to the surface of the rope jacket and in such embodiments sheet layer 3 is not present in the construction. The core 2 with or without sheet layer 3 is fed into the jacket 4 centre during braiding of the strands 5. The rope is now ready for impregnation. Dipping into suitable solution is the most effective method but there are other alternative methods, which involve spraying or wet rollers. The impregnation materials can be solvents of polymers, polyurethane, bitumen or latex or a blend of those materials. Prior to the stretching and heat processing the solvent should be dried out of the rope. A cover 6 can be added at this stage or after the processing. If the core 1 is used without a sheet layer 3 it is advantageous to add such cover 6 prior to the processing but the cover material has to be able to withstand the temperature used in the process. The rope with core is now tensioned and heated up, by means of suitable medium, liquid or air, to the appropriate temperature and simultaneously stretched until it elongates permanently. During the heating, the core 1 shifts from the solid phase to a liquid or semi-liquid phase. The force applied to the axial direction of the rope will partly be transferred into forces working perpendicular to the rope. These perpendicular forces will move the now liquid core material into the inside voids of the rope and fill them up, to the extent that the sheet layer 3 allows the penetration of the core material. If the sheet layer 3 is absent, the core 1 material when in the second phase condition, (typically liquid or semi-liquid phase), will penetrate in-between the strands of the jacket and eventually to the surface of the jacket. If the cover sheet 6 has been applied prior to the process it will stop the fluid core material from entering the surface of the jacket 4. The rope construction is now cooled down and the tension is simultaneously lowered. The rope has now undergone permanent change involving shifting phase of the core and both axial and radial stiffness has been achieved by rearranging the rope sub-elements.

## Claims

1. A method for producing a rope with high stiffness and breaking strength suitable as towing wire for towing fish trawls, the method including:
- firstly providing a thermoplastic core (1) in a solid phase condition,
- secondly, enclosing the core within a sheet layer (3) that has a higher softening point than the core material,
- thirdly, braiding about the core (1) and the sheet layer (3) at least one jacket (4),
- fourthly, changing the phase condition of the core (1) from the first solid phase condition to a second phase condition by heating, and simultaneously stretching said at least one jacket (4) and the core (1) in such a way that the rope becomes permanently elongated,
- subsequently cooling down the rope under tension until the core has regained its solid phase,
wherein the simultaneously stretching of the rope under an appropriate temperature is adapted to elongate the rope permanently and to eliminate vacancies between the core, the sheet layer, and the jacket (4) so that a high stiffness and breaking strength is obtained and axial and radial stiffness are achieved.

2. The method according to claim 1 wherein the second phase condition is a mixture of solid and liquid phase condition.

3. The method of claim 1, wherein changing the phase condition is effected by heating the core to a temperature in the range of 50 - 180° C.

4. The method of claim 3, wherein the core is heated to a temperature in the range of 100 - 130° C.

5. The method of any one of claims 1 to 4, further comprising an additional step of introducing an adhesion material within the at least one jacket prior to the changing of the phase condition of the core.

6. The method according to claim 5, wherein said adhesion material is polyurethane.

7. The method according to claim 5, further comprising removing excess of said adhesion material prior to said stretching step.

8. The method according to claim 7 wherein removing excess of said adhesion material and optionally moisture is conducted by drying in hot air.

## Patentansprüche

1. Verfahren zur Herstellung eines Seils mit hoher Steifigkeit und Reißfestigkeit mit Eignung als Schleppseil für Fischschleppnetze, wobei das Verfahren umfasst:
- erstens Bereitstellen eines thermoplastischen Kerns (1) in einem Festphasenzustand,
- zweitens Umhüllen des Kerns mit einer flächigen Schicht (3), die einen höheren Erweichungspunkt als das Kernmaterial aufweist,
- drittens Umflechten des Kerns (1) und der flächigen Schicht (3) mit mindestens einem Mantel (4),
- viertens Ändern des Phasenzustands des Kerns (1) vom ersten Festphasenzustand zu einem zweiten Phasenzustand durch Erwärmen und gleichzeitig Strecken des mindestens einen Mantels (4) und des Kerns (1) dergestalt, dass das Seil dauerhaft gedehnt wird,
- anschließend Abkühlen des Seils unter Spannung, bis der Kern seine Festphase wiedererlangt hat,
wobei das gleichzeitige Strecken des Seils bei einer geeigneten Temperatur dazu ausgelegt ist, das Seil dauerhaft zu dehnen und Leerstellen zwischen dem Kern, der flächigen Schicht und dem Mantel (4) zu eliminieren, so dass eine hohe Steifigkeit und Reißfestigkeit erzeugt wird sowie eine axiale und radiale Steifigkeit erzielt wird.

2. Verfahren nach Anspruch 1, wobei der zweite Phasenzustand eine Mischung aus Fest- und Flüssigphasenzustand ist.

3. Verfahren nach Anspruch 1, wobei das Ändern des Phasenzustands durch Erwärmung des Kerns auf eine Temperatur im Bereich von 50 bis 180 °C vollzogen wird.

4. Verfahren nach Anspruch 3, wobei der Kern auf eine Temperatur im Bereich von 100 bis 130 °C erwärmt wird.

5. Verfahren nach einem der Ansprüche 1 bis 4, ferner umfassend einen zusätzlichen Schritt zum Einführen eines Adhäsionsmaterials in den mindestens einen Mantel vor dem Ändern des Phasenzustands des Kerns.

6. Verfahren nach Anspruch 5, wobei das Adhäsionsmaterial Polyurethan ist.

7. Verfahren nach Anspruch 5, ferner umfassend: Entfernen von überschüssigem Adhäsionsmaterial vor dem Streckschritt.

8. Verfahren nach Anspruch 7, wobei das Entfernen von überschüssigem Adhäsionsmaterial und optional Feuchte durch Trocknung in heißer Luft vorgenommen wird.

## Revendications

1. Procédé de production d'un cordage avec une grande rigidité et une forte résistance à la rupture approprié comme filin de remorquage pour remorquer des chaluts à poissons, le procédé comportant :
- premièrement, l'obtention d'une âme thermoplastique (1) dans un état de phase solide,
- deuxièmement, l'enfermement de l'âme à l'intérieur d'une couche en feuille (3) qui a un plus haut point de ramollissement que le matériau de l'âme,
- troisièmement, le tressage autour de l'âme (1) et de la couche en feuille (3) d'au moins une gaine (4),
- quatrièmement, la modification de l'état de phase de l'âme (1) du premier état de phase solide à un deuxième état de phase par chauffage, et l'étirage simultané de ladite au moins une gaine (4) et de l'âme (1) de manière à ce que le cordage devienne allongé en permanence,
- ensuite, le refroidissement du cordage sous tension jusqu'à ce que l'âme ait retrouvé sa phase solide,
dans lequel l'étirage simultané du cordage à une température appropriée est adapté pour allonger le cordage en permanence et pour supprimer les vides entre l'âme, la couche en feuille et la gaine (4) de telle sorte qu'une grande rigidité et une forte résistance à la rupture sont obtenues et une rigidité axiale et radiale est atteinte.

2. Procédé selon la revendication 1 dans lequel le deuxième état de phase est un mélange d'état de phase solide et liquide.

3. Procédé de la revendication 1, dans lequel la modification de l'état de phase est effectuée par chauffage de l'âme jusqu'à une température dans la gamme de 50-180 °C.

4. Procédé de la revendication 3, dans lequel l'âme est chauffée jusqu'à une température dans la gamme de 100-130 °C.

5. Procédé de l'une quelconque des revendications 1 à 4, comprenant en outre une étape supplémentaire d'introduction d'un matériau adhésif à l'intérieur de l'au moins une gaine avant la modification de l'état de phase de l'âme.

6. Procédé selon la revendication 5, dans lequel ledit matériau adhésif est le polyuréthane.

7. Procédé selon la revendication 5, comprenant en outre le retrait de l'excès dudit matériau adhésif avant ladite étape d'étirage.

8. Procédé selon la revendication 7, dans lequel le retrait de l'excès dudit matériau adhésif et éventuellement de l'humidité est effectué par séchage dans de l'air chaud.
